

June 8, 1937.

R. M. PFALZGRAFF

2,083,395

METHOD OF MAKING CORES FOR ELECTRICAL APPARATUS

Filed Aug. 14, 1935



Inventor:  
Ross M. Pfalzgraff,

by Harry E. Dunham

His Attorney.

## UNITED STATES PATENT OFFICE

2,083,395

## METHOD OF MAKING CORES FOR ELECTRICAL APPARATUS

Ross M. Pfalzgraff, Lynn, Mass., assignor to  
General Electric Company, a corporation of  
New York

Application August 14, 1935, Serial No. 36,103

1 Claim. (Cl. 22—203)

My invention relates to a method of making cores for electrical apparatus of the type including a laminated core structure having a frame cast thereon.

5 In making cores for electrical apparatus in which the laminations are retained in assembled relation by a metal frame cast about the periphery of the laminations, difficulty is encountered in obtaining satisfactory castings, as the frames are 10 likely to crack unless some provision is made to allow for the shrinkage of the metal frame during cooling.

An object of my invention is to provide an improved core for electrical apparatus comprising 15 assembled laminations secured in a metal frame cast about the edge of the laminations and constructed in such manner as to minimize shrinkage cracks in the cast metal.

Another object of my invention is to provide an 20 improved method of making a core for electrical apparatus by casting a metal frame about the edge of assembled laminations in such manner as to minimize shrinkage cracks in the cast metal.

My invention will be more fully set forth in the 25 following description referring to the accompanying drawing and the features of novelty which characterize my invention will be pointed out with particularity in the claim annexed to and forming a part of this specification.

30 For a better understanding of my invention, reference is made to the accompanying drawing, wherein Fig. 1 is a perspective view, partly in section, of a stator core embodying my invention; Fig. 2 is an enlarged fragmentary sectional view 35 of assembled laminations clamped together and illustrating the axially spread edge thereof; Fig. 3 is a sectional view of the assembled core and casting mold.

Referring to the drawing, I have shown my invention in connection with the stationary member 40 of a dynamo-electric machine including a laminated magnetic core structure 18 having a series of teeth 11 providing slots 12, in which any suitable windings may be placed. This core structure 45 is secured in a continuous thin frame 13, of iron or other metal, cast in direct contact with the entire outer edge or peripheral surface 14 and with the adjacent sides 15 and 16 of the laminated core 18, for clamping the laminations in assembled relation.

In manufacturing such a stationary member, I 50 have found that some provision must be made to allow for shrinkage of the cast frame both axially and radially to prevent the development of cracks in the cast metal upon cooling. I assem-

ble the laminations 10 and clamp them in the desired relation by annular clamping rings 17 having their outer periphery just beyond the base portions of the teeth 12 and extending inwardly slightly beyond the mid portion of the teeth. 5 These clamping rings are secured together by bolts 18 arranged in the slots 11 and out of contact with the bottom of the slots, so as to permit a certain amount of radial shrinkage on cooling of the cast frame 13. The clamping pressure on the inner edge of the laminations is adjusted by tightening the nuts 19 on the bolts 18, so as to cause the other edge of the laminations to spread apart axially, as illustrated in Fig. 2. This axially spread edge of the laminations is compressible and allows for axial shrinkage of the cast frame when it cools. Around this axially spread edge and the adjacent sides of the laminations is arranged, as shown in Fig. 3, a mold 20, which may be of the permanent type or of such material as molding sand, and which cooperates with upper and lower cores 21 to form the complete mold for the cast frame. This mold is supported by a flask 22 and arranged between top and bottom boards 23 and 24 held together by clamps 25. The clamping rings 17 are of such size that they just cover the slots 11 and the use of a sand mold between these rings and the molding space provides a yieldable cushion which permits radial shrinkage of that portion of the cast frame extending beyond the laminations. The top board 23 is provided with an opening 26, communicating with the gate 27, into which the metal is poured in casting the frame 13. Thus, it is readily seen that I provide a core structure for electrical apparatus utilizing assembled laminations retained in the desired relation by a continuous metal frame cast in direct contact with an edge and the adjacent sides of the laminations, and provide a method of making the same which allows for both radial and axial shrinkage of the cast frame, thereby preventing the formation of cracks in the finished product.

Although I have shown my invention in connection with a dynamo-electric machine, it is apparent that it can be used in other types of electrical apparatus utilizing laminated core structures and modifications of the embodiment of my invention illustrated and described will be apparent to those skilled in the art. I desire it to be understood, therefore, that my invention is not to be limited to the particular arrangement disclosed, and I intend, in the appended claim to cover all modifications which do not depart from the spirit and scope of my invention.

What I claim as new and desire to secure by Letters Patent of the United States is:

The method of making a core for electrical apparatus which consists of assembling a group of 5 annular laminations having a series of slots in one edge thereof, clamping together said slotted edge by clamping rings secured by means out of contact with the bottom of said slots in said laminations to permit radial shrinkage of said lami-

nations and under such pressure as to cause the other edge of said laminations to spread axially, forming a mold with a molding space about said spread edge of said assembled laminations and a yieldable portion of the mold between said clamping rings and said molding space, and casting a metal frame in contact with said assembled laminations in said molding space. 5

ROSS M. PFALZGRAFF.